

**1**

3,105,500

**SOIL RETAINING FINISH FOR TEXTILES**

Abraham Wilson, Millstone, William Julius van Loo, Jr., Middlesex, and Frank M. Cowen, North Plainfield, N.J., assignors to American Cyanamid Company, New York, N.Y., a corporation of Maine  
No Drawing. Filed Aug. 4, 1959, Ser. No. 831,489  
9 Claims. (Cl. 131—208)

This invention relates to the treatment of fibrous and related materials. More particularly, it relates to a process for imparting a durable soil-attracting and soil-retaining finish to fibrous, shredded, cellular and related materials by treatment with a composition containing a long-chain anion active material and a long-chain cation active material.

It is an object of the present invention to provide a treatment for materials which will result in increased absorption of soil, more efficient pick-up of soil and better soil retaining or holding ability than untreated materials.

It is a further object of the present invention to provide a process for treating filter materials to improve the removal of solids, liquids or gaseous materials from a fluid or gaseous medium.

A further object of the present invention is to provide a process for imparting a durable soil-attracting and soil-retaining finish to fibrous materials, particularly durable to washing or laundering. Here it should be noted that known soil scavengers, such as oils and waxes, are not durable to laundering.

It is a still further object of the present invention to provide a composition which when applied to fibrous materials imparts soil-attracting and soil-retaining properties thereto which is comparatively easy to prepare and to employ.

Still further, it is an object of the present invention to provide various fibrous materials having a durable soil-attracting and soil-retaining finish thereon and more specifically such materials as cigarette filters or filters normally employed in the manufacture of cigarettes.

These and other objects and advantages of the present invention will become more apparent from the detailed description thereof set forth hereinbelow.

In accordance with the present invention we have found that these and other objects and advantages may be obtained by treating fibrous, shredded, cellular and related materials with a composition containing long-chain anions and long-chain cations.

The term "fibrous" employed herein and throughout the present specification and claims is intended to include fibers or materials formed therefrom, whether they be of vegetable, animal or of synthetic origin or mixtures of two or more of such materials. As illustrative of vegetable fibrous materials, those of cotton, jute, hemp, ramie, linen and the like may be mentioned. Wool is illustrative of animal fibers, while synthetic fibers may be typified by nylon, viscose rayon, cellulose acetate, polyester fibers, available commercially as Dacron, and acrylic fibers, such as are available commercially as Creslan, Orlon and Acrilan, may be mentioned.

As indicated, "fibrous" as employed herein may apply to the fibers themselves or fabrics and articles formed therefrom. In the case of fabrics, they may be knitted,

**2**

woven, non-woven, felted or otherwise formed and may be suitable for a wide variety of end uses.

Of the possible fibrous materials contemplated, cellulosic materials, and in particular those containing a substantial percentage of cotton, as, for example, at least 50%, and cellulose acetate have resulted in particularly good results.

The term "long-chain" as applied herein in reference to anions and cations is intended to refer to aliphatic chains containing between 8 and 30 carbon atoms, and in the case of alkyl-aryl compounds of the benzene series between about 4 and 26 carbon atoms. Where the aryl group is naphthalene, the alkyl group may contain between 0 and about 22 carbon atoms. These or their equivalent materials may be employed. Essentially the materials suited for use in the preparation of the soil retaining finish are anion and cation active materials characterized by surface activity and capable of combining with one another, usually and preferably to form an insoluble precipitate in water.

20 The anion and cation active materials may be derived from anionic and cationic surface-active agents or surfactants. These materials are well known and have been described heretofore for various purposes, including wetting, penetrating, emulsifying, dispersing, solubilizing, foaming, frothing and washing or scouring in addition to other uses.

The anionic active agents may be divided into the following major classes:

30 Alkyl aryl sulfonates  
Alkyl sulfates  
Alkyl sulfonates  
Sulfated and sulfonated amides and amines  
Sulfated and sulfonated esters and ethers

35 Among the many anionic surface active agents which may be the source for the long-chain anions are the following:

Sodium bis(tridecyl)-sulfosuccinate  
40 Sodium N-methyl-N-oleoyl taurate  
Oleic acid ester of sodium isethionate  
Sodium lauryl sulfate  
Disodium bis(sulfonaphthyl)-methane  
Sodium octylphenoxy polyglycol sulfonate  
45 Sodium alkylbenzenesulfonate  
Sodium isopropylnaphthalenesulfonate  
Sodium heptadecyl sulfate  
Polyoxyethylene sorbitan monostearate

50 The cationic-active agents may be divided into the following major classes:

Salts of simple primary and tertiary amines  
Quaternary ammonium salts  
Salts and quaternary derivatives of amino acids  
55 Salts and quaternary derivatives of imidazolines  
Salts and quaternary derivatives of amino esters

Among the many cationic surface-active agents which may be the source for the long-chain cations are the following:

60 Dimethyl benzyl cetyl ammonium chloride  
Dimethyl 2-hydroxyethyl stearamidopropylammonium nitrate  
Dimethyl benzyl stearamidopropyl ammonium chloride

Lauramidopropyl dimethyl carboxyethyl ammonium betaine

1-hydroxyethyl 2-heptadecyl glyoxalidine

Mixture of octadecylamine and octadecylguanidine salts of octadecylcarbamic acid, reacted with ethylene oxide

It will be apparent that mixtures of two or more anionic-active agents and two or more cationic-active agents may be employed in accordance with the present invention.

In one of the methods of treating fibrous materials in accordance with the present invention, the anionic-and cationic-active agents are reacted in aqueous solution using essentially equimolar amounts of the reactants. When the reaction product consisting of long-chain anionic and long-chain cationic portions is sufficiently insoluble in water, it may be separated by physical means, as, for example, filtration. When the product is too soluble in the aqueous medium for isolation by physical separation, as for example, filtration, it may be separated by extraction with a water-insoluble organic solvent in which the product is itself soluble. The organic solvent may then be evaporated to give the desired end-product. In either case, the solution of the isolated product in a non-aqueous solvent, such as alcohol or acetone, is applied to the fibrous material, which is then dried and/or cured.

In a second method, a non-aqueous solution of essentially equimolecular amounts of the anionic-and cationic-active agent is supplied to the fibrous material, which is then dried and/or cured. In accordance with this technique, it is believed that the soil-attracting and/or soil-retaining finish is formed in situ on the fibrous material, the reaction between the materials being effected during the drying and removal of the solvent from the surface having been finished.

In a third method, the anionic- and cationic-active agents are applied consecutively in non-aqueous solution to the fibrous material to be finished. Although the application may be in either order, it is believed more advantageous to apply the cationic agent first, since the cationic agent appears to have greater affinity for the fibrous material, especially if it is of cellulosic nature.

Generally speaking, the first and second of the above-described methods give approximately the same results and are preferred. The third is believed to be less satisfactory due to the leaching of the first component from the fibrous substrate by the solvent employed for the second component.

While it is generally recommended that equimolecular amounts of anionic and cationic agents be employed in preparing the soil-retaining finishing material, slight excesses of either of the components are permissible. An excess of one over the other, however, is economically disadvantageous and, in general, should be avoided. Additionally, substantial excesses of one of the components over the other may result in the formation of a colloidal solution, preventing the isolation of the product by simple physical separation means, as, for example, filtration. In general, this difficulty is overcome by employing equimolecular amounts of reactants and by reacting at a low temperature.

Suitable non-aqueous solvents for use in applying the long-chain anionic-cationic products to the fibrous materials include ethanol, isopropanol and acetone. However, other suitable alcohols, ketones, esters, ethers and the like may be employed. The use of water as the solvent where the product is sufficiently soluble in water in general produced less satisfactory results with respect to the durability of the finish to laundering.

The composition of the present invention or the components thereof may be applied to suitable fibrous material by any of the conventional means, such as dipping, spraying, immersing, padding or the like.

In general, the soil-retaining property of the treated

75

material is increased as the amount of the finishing composition of this invention increases on the material. Below a concentration of about 0.5% on the dry weight of the material there is relatively little improvement over the untreated material. In general, an application of at least 2% is recommended; however, the amount applied will depend on the nature of the material being treated. Also, the effectiveness of the treatment and its durability to washing is to some extent dependent upon the choice of anionic and cationic components. Thus, anionic and cationic components which result in the formation of a product having a low solubility in water so as to be capable of being characterized as being substantially water-insoluble are more durable to washing than those having greater solubility in water.

After application of the soil-retaining finish to a suitable fibrous substrate, the material is preferably dried, resulting in the evaporation of the solvent medium, and thereafter cured into intimate association with the fibrous substrate. Curing may be effected at temperatures on the order of from between about 250° to about 350° for periods of time of from about ten minutes to about five minutes, respectively. In general, curing of the finish on the substrate improves the soil-retaining ability of the finish and is greatly preferred. It should be noted that the above temperatures and times are merely illustrative with respect to curing conditions and that in general curing times and temperatures may be varied over wide limits to achieve good results.

In order to illustrate the present invention, the following examples are given primarily by way of illustration. No details or enumerations contained therein should be construed as limitations on the present invention, except insofar as they appear in the appended claims. All parts and percentages are by weight, unless otherwise clearly indicated.

#### EXAMPLE 1

*Dimethyl 2-Hydroxyethyl Stearamidopropyl Ammonium Bis(Tridecyl)-Sulfosuccinate*



Solution A was prepared by dissolving 84 parts (0.153 mole) of sodium bis(tridecyl)-sulfosuccinate in 2,716 parts of water while stirring and heating to 67° C. Solution B was prepared by dissolving 73 parts (0.153 mole) of dimethyl 2-hydroxyethyl stearamidopropyl ammonium nitrate in 588 parts of water at 35° C. while stirring. Solution B was slowly added to solution A while the latter was cooled in an ice bath. At about 20° C. a white, waxy precipitate was formed, which was separated by filtration and washed with water. The wax-like product was dried in vacuo at 65° C. to a solids content of about 95%.

#### EXAMPLE 2

The product of Example 2 was prepared by a process similar to that of Example 1 with substitution of an equivalent amount of dimethyl-2-hydroxyethyl stearamidopropyl ammonium phosphate for the nitrate used in Example 1.

#### EXAMPLE 3

Solution A was prepared by dissolving 73 parts (0.153 mole) of dimethyl 2-hydroxyethyl stearamidopropyl ammonium nitrate in 33.6 parts of alcohol. Solution B was prepared by dissolving 84 parts (0.153 mole) of sodium bis(tridecyl)-sulfosuccinate in 84 parts of alcohol. Solution B was added to solution A at room temperature, and stirring was continued for 15 minutes. The resulting solution was clear with no precipitate and contained 50% of the product of Example 1 on the weight of the solution.

(When the above solution was diluted with water and

the precipitate was filtered off and dried, the product was similar to that of Example 1.)

#### EXAMPLES 4-7

Equimolecular amounts of anionic and cationic surface active agents in aqueous solutions were combined. The aqueous reaction mixture was extracted with ethyl acetate or methyl ethyl ketone, and the product was recovered by distilling off the solvent. The quantities used are shown in Table I below.

TABLE I

| Example No. | Anionic Agent          |               |                                 | Cationic Agent         |               |                                 |
|-------------|------------------------|---------------|---------------------------------|------------------------|---------------|---------------------------------|
|             | Name<br>(See<br>Below) | Parts<br>Used | Total<br>Parts<br>with<br>Water | Name<br>(See<br>Below) | Parts<br>Used | Total<br>Parts<br>with<br>Water |
| 4-----      | A                      | 13.8          | 300                             | E                      | 10.0          | 45                              |
| 5-----      | B                      | 9.6           | 200                             | E                      | 10.0          | 45                              |
| 6-----      | C                      | 8.3           | 50                              | F                      | 10.0          | 80                              |
| 7-----      | D <sup>a</sup>         | 12.0          | 100                             | F                      | 10.0          | 80                              |

A—Sodium bis(tridecyl)-sulfosuccinate.  
B—Oleic acid ester of sodium isethionate.  
C—Sodium N-methyl-N-oleyl taurate.  
D—Mixture of octadecylamine salt of octadecylcarbamic acid, and octadecylguanidine salt of octadecylcarbamic acid reacted with ethylene oxide.  
E—Dimethyl benzyl ethyl ammonium chloride.  
F—Dimethyl 2-hydroxyethyl stearamidopropyl ammonium nitrate.

<sup>a</sup> Anionic agent D is usually identified as a cationic agent. However, it is believed that an exchange takes place in the cationic portion thereof with the second cationic agent, to give a new and more durable (less soluble) salt.

#### EXAMPLES 8-10

Ethanol solutions containing an anionic and a cationic surface active agent at a 1:1 molar ratio were prepared. The quantities used, on 100% real basis, are shown in Table II. Also shown are the strengths of the solutions in terms of percent organic salt on weight of solution.

These examples correspond in composition to those of Examples 4-7 (Table I) as follows:

|                        |            |
|------------------------|------------|
| Example 4              | Example 8  |
| Example 5 <sup>1</sup> | Example 9  |
| Example 6              | Example 10 |
| Example 7              |            |

<sup>1</sup> One of the components in Example 5 was too insoluble in ethanol for it to be used in this method of preparation.

TABLE II

| Example No. | Anionic Agent     |       | Cationic Agent    |       | Total<br>Parts<br>with<br>Ethanol | Solution<br>Strength,<br>percent <sup>2</sup> |
|-------------|-------------------|-------|-------------------|-------|-----------------------------------|-----------------------------------------------|
|             | Name <sup>1</sup> | Parts | Name <sup>1</sup> | Parts |                                   |                                               |
| 8-----      | A                 | 0.58  | E                 | 0.42  | 50                                | 2.00                                          |
| 9-----      | C                 | 0.28  | F                 | 0.34  | 50                                | 1.24                                          |
| 10-----     | D                 | 0.38  | F                 | 0.32  | 50                                | 1.40                                          |

<sup>1</sup> For identification see Table I.

<sup>2</sup> Percent organic salt in solution.

#### EXAMPLES 11-14

Aqueous solutions or dispersions of equimolecular amounts of anionic and cationic agents were prepared. The quantities used, on 100% real basis, are shown in Table III.

These examples correspond in composition to those of Examples 4-7 (Table I) as follows:

|           |            |
|-----------|------------|
| Example 4 | Example 11 |
| Example 5 | Example 12 |
| Example 6 | Example 13 |
| Example 7 | Example 14 |

6  
TABLE III

| Example No. | Anionic Agent     |       | Cationic Agent    |       | Total<br>Parts<br>with<br>Water | Solution<br>Strength,<br>percent <sup>2</sup> |
|-------------|-------------------|-------|-------------------|-------|---------------------------------|-----------------------------------------------|
|             | Name <sup>1</sup> | Parts | Name <sup>1</sup> | Parts |                                 |                                               |
| 11-----     | A                 | 0.58  | E                 | 0.42  | 50                              | 2.0                                           |
| 12-----     | B                 | 0.49  | E                 | 0.51  | 50                              | 2.0                                           |
| 13-----     | C                 | 0.46  | F                 | 0.55  | 50                              | 2.0                                           |
| 14-----     | D                 | 0.51  | F                 | 0.49  | 50                              | 2.0                                           |

<sup>1</sup> For identification see Table I.

<sup>2</sup> Percent organic salt in solution.

#### EXAMPLE 15

An approximately 3% application of the product of Example 2 was made on viscose rayon carpet by padding with an approximately 3% solution of the product of Example 2 in ethanol (6 parts of product in 200 parts of ethanol) with a pick-up of 100% based on the weight of the carpet. The carpet was dried.

The washes referred to in Table IV were carried out at 140° F. in a Laundromat washing machine with neutral soap according to a standard procedure.

The soiling test using a drum type laboratory soiler and a synthetic soil was carried out by the procedure described in the American Dyestuff Reporter 45, 190 (1956). The results are shown in Table IV below.

30

TABLE IV

#### Soiling Test Results

| Washes: | Soiling index <sup>1</sup> |
|---------|----------------------------|
| 0-----  | 5.17                       |
| 1-----  | 5.95                       |
| 5-----  | 5.18                       |

<sup>1</sup> The "Soiling Index" is defined in the following manner:

$$40 \quad \text{Soiling index} = \frac{\text{Apparent soil of treated fabric}}{\text{Apparent soil of untreated fabric}}$$

45 and

$$\text{Apparent soil} = \frac{(1-R_s)^2}{2R_s} - \frac{(1-R_u)^2}{2R_u}$$

Where  $R_s$  and  $R_u$  are the fraction of light reflected from soiled and unsoiled test pieces, respectively. Thus, a soiling index of 1.0 or greater indicates that the treated fabric has an equal or greater affinity for soil than the untreated fabric.

#### EXAMPLE 16

55 Viscose carpet was treated with a 2% solution of the product of Example 1 in ethanol using a 100% pick-up on the weight of the carpet. The treated carpet was dried for one hour at 225° F.

The soiling test was carried out as described in Example 15. The treated carpet had a soiling index of 4.81.

60

#### EXAMPLE 17

Cotton flannel cloth was treated with various amounts of the product of Example 1. The applications were made from solutions in alcohol with approximately a 100% pick-up on the weight of the fabric. All of the fabrics were dried for 30 minutes at 225° F., and some of the fabrics were cured for 6 minutes at 290° F., as indicated in Table V. Also, as indicated, some of the treated fabrics were washed for 20 minutes in a Laundromat washer with soap and 140° F. water. Portions of all the fabrics were then soiled by the standard procedure described in Example 15. The reflectance measurements 75 of the fabrics before and after soiling were then deter-

mined and the soiling indices were calculated, as described in Example 15. The results are shown in Table V.

TABLE V

| Fabric Treatment, percent | Washes | Cured at 290° F. | Soiling Index |
|---------------------------|--------|------------------|---------------|
| 5                         | None   | Yes              | 4.05          |
| 2                         | None   | Yes              | 2.65          |
| 1                         | None   | Yes              | 1.56          |
| 0.5                       | None   | Yes              | 1.05          |
| 0.1                       | None   | Yes              | 1.14          |
| 0.01                      | None   | Yes              | 1.14          |
| 2                         | None   | No               | 2.11          |
| 2                         | None   | Yes              | 2.69          |
| 2                         | 1      | Yes              | 1.53          |
| 2                         | 2      | Yes              | 1.39          |
| 2                         | 3      | Yes              | 1.60          |
| 2                         | 4      | Yes              | 1.44          |
| 2                         | 5      | Yes              | 1.28          |

The data in Table V indicates that the degree of soiling depends upon the concentration of the agent on the fabric, the soiling scavenging effect at concentrations of 0.5% or less being negligible. The initial scavenging effect is improved by curing the dried fabric at 290° F. Applications of 2% or more of the agent are effective after five washes.

## EXAMPLE 18

Viscose carpet was treated with 1% solutions of the product of Example 1 in various solvents. The solutions were prepared in two ways: in Method A the dry product was dissolved in the solvent; in Method B a 50% stock solution in ethanol was diluted with the solvent chosen. The pick-up on the weight of the carpet was approximately 100%. The washing was done by the procedure of Example 15. The soiling index was determined as described in Example 15. The results are shown in Table VI.

TABLE VI

| Solvent     | Method of Solution | Washes | Soiling Index |
|-------------|--------------------|--------|---------------|
| Ethanol     | A                  | 0      | 4.95          |
| Do.         | B                  | 5      | 4.98          |
| Isopropanol | A                  | 5      | 1.12          |
| Do.         | B                  | 0      | 4.98          |
| Acetone     | A                  | 0      | 5.57          |
| Do.         | B                  | 5      | 1.14          |

## EXAMPLE 19

One percent applications of the products of Example 1 (in alcohol) and Example 3 (on solids basis) were applied to cotton flannel and the soiling test of Example 15 was applied to the treated fabrics. The results are shown in Table VII.

TABLE VII

## Comparison of Products Prepared by Two Methods

| Product:  | Soiling |
|-----------|---------|
| Example 1 | 1.76    |
| Example 3 | 1.74    |

The examples serve to show that the products made by the procedures of Examples 1 and 3 give substantially the same results on cotton flannel.

## EXAMPLE 20

Cotton flannel was treated with 2% solutions of the products of Examples 4-7 in ethanol, using a 100% pick-up on the weight of the fabric. The treated fabrics were dried at 200° F. for 6 minutes and cured at 300° F. for 6 minutes. The washings were carried out in a Laundromat washer with soap and 140° F. water by the standard procedure. The fabrics were soiled by the standard

procedure of Example 15. The results are shown in Table VIII.

TABLE VIII

| 5  | Product   | Soiling Index |        |          |
|----|-----------|---------------|--------|----------|
|    |           | Initial       | 1 Wash | 3 Washes |
| 10 | Example 4 | 1.89          | 1.65   | 2.06     |
|    | Example 5 | 1.75          | 1.30   | 1.80     |
|    | Example 6 | 1.73          | 1.97   | 1.15     |
|    | Example 7 | 1.48          | 1.46   | 1.27     |

<sup>1</sup> This product was not durable to laundering, although the corresponding composition of Example 9 was durable (Table X).

## EXAMPLE 21

Cotton flannel was treated with 2% solutions or dispersions of the products of Examples 4-7 in water, using a 100% pick-up on the weight of the fabric. The treated fabrics were dried at 225° F. for 10 minutes and cured at 290° F. for 6 minutes. Washings were carried out in 100° F. water with soap and soda ash present. The fabrics were soiled by the procedure of Example 15. The results are shown in Table IX.

| 25 | Product   | Soiling Index |        |          |
|----|-----------|---------------|--------|----------|
|    |           | Initial       | 1 Wash | 3 Washes |
| 30 | Example 4 | 2.34          | 1.06   | 1.13     |
|    | Example 5 | 2.79          | 0.97   | 1.05     |
|    | Example 6 | 2.45          | 0.91   | 0.98     |
|    | Example 7 | 1.97          | 1.03   | 0.97     |

These examples serve to show that aqueous applications of the products of Examples 4-7 are not durable to laundering.

## EXAMPLE 22

The alcoholic solutions of Examples 8-10 were applied to cotton flannel with a 100% pick-up on the weight of the fabric. The fabrics were dried and cured as in Example 20. The washings and soiling tests were carried out as in Example 20. The results are shown in Table X.

| 40 | Product    | Percent application | Soiling Index |        |          |
|----|------------|---------------------|---------------|--------|----------|
|    |            |                     | Initial       | 1 Wash | 5 Washes |
| 45 | Example 8  | 2.00                | 1.65          | 1.57   | 1.69     |
|    | Example 9  | 1.24                | 1.61          | 1.57   | 1.40     |
|    | Example 10 | 1.40                | 1.80          | 1.44   | 1.39     |

Table X illustrates that applications of the soil-retaining finishing composition of this invention from alcoholic solutions is durable up to 5 launderings.

## EXAMPLE 23

The aqueous solutions of Examples 11-14 were applied to cotton flannel with a 100% pick-up on the weight of the fabric. The treated fabrics were dried at 225° F. for 10 minutes and cured at 290° F. for 6 minutes. The washings were carried out in 100° F. water with soap and soda ash present. The fabrics were soiled by the procedure of Example 15. The results are shown in Table XI below.

| 50 | Product    | Soiling Index |        |          |
|----|------------|---------------|--------|----------|
|    |            | Initial       | 1 Wash | 5 Washes |
| 55 | Example 11 | 1.75          | 1.13   | 1.05     |
|    | Example 12 | 1.40          | 1.04   | 1.05     |
|    | Example 13 | 1.65          | 0.92   | 0.80     |
|    | Example 14 | 1.77          | 1.13   | 1.00     |

These examples serve to show that applications of the non-isolated products of Examples 4-7 are not durable to laundering when applied from aqueous solution.

#### EXAMPLE 24

Applications of the product of Example 1 and of each of the surface active agents used in preparing it were made on cotton flannel using 2% solutions in ethanol, and a 100% pick-up on the weight of the fabric. The treated fabrics were dried for 30 minutes at 50° F. and cured for 6 minutes at 290° F. The washings and soiling tests were done as described in Example 17. The results are shown in Table XII.

TABLE XII

| Product                           | Washes | Soiling Index |
|-----------------------------------|--------|---------------|
| Example 1.....                    | 0      | 2.69          |
| Do.....                           | 1      | 1.53          |
| Do.....                           | 2      | 1.39          |
| Anionic Agent <sup>1</sup> .....  | 0      | 1.78          |
| Do.....                           | 1      | 0.94          |
| Do.....                           | 2      | 1.00          |
| Cationic Agent <sup>2</sup> ..... | 0      | 1.88          |
| Do.....                           | 1      | 1.24          |
| Do.....                           | 2      | 1.18          |

<sup>1</sup> Anionic Agent: sodium bis(tridecyl)-sulfosuccinate.

<sup>2</sup> Cationic Agent: dimethyl 2-hydroxyethyl stearamidopropyl ammonium nitrate.

This example serves to show that the anionic and cationic agents used in preparing the product of Example 1, when used separately, impart less soil-retaining properties to cotton flannel than the product of Example 1.

#### EXAMPLE 25

Applications of 1% and 2% solids of the products of Example 1 on the weight of the fabric were made to spun acetate from alcohol. Strips, 10.5 cm. x 4 cm. were taken, rolled into a tight pack, inserted in glass tubes and cigarettes attached. The cigarettes were smoked by means of a smoking apparatus consisting of a flask with a suction bulb and water as a metering liquid. Ten puffs of 35 ml. at 30-second intervals were made on each cigarette. Several cigarettes were smoked through the same filter, and the weight pick-up was taken at intervals after desiccating for 25 hours. This weight was taken as a measure of the tars and/or solids picked up. In Table XIII, the tar and/or solids pick-up of the treated acetate is compared with that of untreated acetate or untreated acetate padded through alcohol only.

TABLE XIII

| No. of Cigarettes<br>Through Same<br>Filter | Tar and/or Solids Pick-up (Percent O.W.F.) |         |                      |       |    |
|---------------------------------------------|--------------------------------------------|---------|----------------------|-------|----|
|                                             | Untreated                                  | Alcohol | Product of Example 1 |       | 2% |
|                                             |                                            |         | 1%                   | 2%    |    |
| 2.....                                      | 1.61                                       | 1.03    | 4.79                 | 2.79  |    |
| 6.....                                      | 3.95                                       | 7.45    | 14.60                | 11.50 |    |
| 12.....                                     |                                            | 16.8    | 26.6                 | 17.6  |    |
| 18.....                                     |                                            | 26.4    |                      | 27.2  |    |

As will be seen from the above examples and disclosure, the present invention has wide-spread utility. Thus, the present process may be employed for the treating of a number of articles or materials capable of being converted to a number of articles, wherein soil attraction and retention is highly desirable. As examples of suitable end-products, fibrous doormats, dust cloths, dust mops, wiping cloths, wood-cellulose products, sponges, both natural and synthetic, are illustrative.

Further industrial and domestic applications include the use of the soil-retaining finish in elements in air-conditioners and furnace filters to improve filtration properties and possibly effect the better removal of pollen and absorption of odors.

The utility in such specific applications as cigarette filters is clearly demonstrated in Table XIII, where it is shown that the 1% applications level absorption is substantially three times better than the untreated cellulose acetate.

It will be noted that other materials which are compatible with the essential components of the present composition may be employed therewith. Thus, for example, disinfectants, perfumes, coloring agents, and the like may be employed in compositions insofar as they do not interfere with or impair significantly the soil-retaining and attracting properties of the finish.

We claim:

1. A process for imparting a durable soil retaining finish to fibrous materials which comprises applying thereto, from a non-aqueous solvent, as a soil retaining finish from about 2 to about 5% of an essentially equimolecular amount of a long chain anionic surface active component and a long chain cationic surface active component, said anionic and cationic component having about 13 to about 18 carbon atoms, and thereafter drying and curing said finish on said fibrous material.

2. A process for imparting a durable soil retaining finish to fibrous materials which comprises applying thereto, from a non-aqueous solvent, from about 2 to about 5% of a composition containing essentially equimolecular amounts of a long chain anionic surface active component and a long chain cationic surface active component, said anionic and cationic component having about 13 to about 18 carbon atoms, and thereafter drying and curing said component on said fibrous material to react the anionic and cationic components to form the soil retaining finish.

3. A process for imparting a durable soil retaining finish to fibrous materials which comprises applying thereto, from a non-aqueous solvent solution, as a soil retaining finish from about 2 to about 5% of the water insoluble reaction product of essentially equimolecular amounts of a long chain anionic surface active component and a long chain cationic surface active component, said anionic and cationic component having about 13 to about 18 carbon atoms, and thereafter drying and curing the said finish on said fibrous material.

4. Fibrous material having as a durable soil retaining finish thereon from about 2 to about 5% of a water insoluble reaction product of essentially equimolecular amounts of a long chain anionic surface active component and a long chain cationic surface active component, said anionic and cationic component having about 13 to about 18 carbon atoms, said water insoluble reaction product having been applied from a non-aqueous solvent solution.

5. Fibrous material according to claim 4 containing cellulose.

6. Fibrous material according to claim 4 containing cellulose acetate.

7. Fibrous material according to claim 4 in which the material is formed cotton fabric.

8. A cigarette filter impregnated with at least 0.5% of a water insoluble reaction product of essentially equimolecular amounts of a long chain anionic surface active component and a long chain cationic surface active component, said anionic and cationic component having from about 13 to 18 carbon atoms, said reaction product having been applied to said cigarette filter material from a non-aqueous solvent solution.

9. A soil retaining composition comprising at least 2% solids of a water insoluble reaction product of essentially equimolecular amounts of a long chain anionic surface active component and a long chain cationic surface active component, said anionic and cationic component having

11

from about 13 to about 18 carbon atoms, and a non-aqueous solvent therefor.

## References Cited in the file of this patent

## UNITED STATES PATENTS

|           |           |                |
|-----------|-----------|----------------|
| 2,051,843 | Gotte     | Aug. 25, 1936  |
| 2,482,816 | Van Mater | Sept. 27, 1949 |

|             |
|-------------|
| 2,693,430   |
| 2,739,598   |
| 2,746,928   |
| 2,763,267   |
| 5 2,780,228 |

12

|                |                |
|----------------|----------------|
| Cross et al.   | Nov. 2, 1954   |
| Eirich         | Mar. 27, 1956  |
| Darragh et al. | May 22, 1956   |
| Muller         | Sept. 18, 1956 |
| Touey          | Feb. 5, 1957   |

## FOREIGN PATENTS

|         |               |
|---------|---------------|
| Belgium | Mar. 15, 1951 |
|---------|---------------|